

## UNITED STATES PATENT OFFICE

2,062,818

## MOLDING SAND

Roy E. Paine, Cleveland, Ohio, assignor to Aluminum Company of America, Pittsburgh, Pa., a corporation of Pennsylvania

No Drawing. Application November 20, 1934,  
Serial No. 753,900

7 Claims. (Cl. 22—188)

This invention relates to providing a molding sand composition which is adapted to the production of green sand molds wherein aluminum-magnesium alloys may be cast without any unfavorable reaction between the metal and the atmosphere or the components of the molding composition.

In the art of casting easily oxidizable metals in green sand molds, which are herein defined to be molds made from water tempered sand, considerable difficulty has been encountered because of the reaction between the metal and the water in the molding sand. This reaction results in the formation of a heavy oxide skin or dross on the surface 5 of the metal which may interfere with the flow of metal in the mold. The dross is also likely to adhere to the casting and produce a rough unsatisfactory surface. In the case of certain alloys the reaction may occur below the surface of the casting the result of which cannot be seen by ordinary inspection. Various expedients have been tried in an effort to eliminate water from the mold, for example, such practices as drying the mold before introducing the metal, or using 10 a non-aqueous binder have been employed, but they either add to the cost of producing castings or impair the molding characteristics of the sand. An extensive search has therefore been made to find more practicable means of overcoming the ill 15 effect of water upon the metal poured in a green sand mold.

The casting of aluminum-magnesium alloys in molds made from water tempered sand presents a peculiarly difficult problem because of the formation 20 of a porous black ring or "frame" immediately below the surface of the casting. The occurrence of frame is definitely associated with the presence of water since it does not appear in castings produced in either dry or non-aqueous tempered sand molds. The occurrence of frame is undesirable 25 for the reason that it creates a porous zone below the surface of the casting and thereby reduces the cross sectional area of sound metal which in turn diminishes the strength of the article. This deleterious effect is especially evident in thin sections of a casting where any decrease in the thickness is likely to result in an early failure in service.

Oxidation inhibitors have been employed in the production of sand molds for casting magnesium 30 base alloys and it might therefore appear logical that the substances commonly used to protect such alloys against burning in sand molds would afford protection for aluminum base alloys containing magnesium. Experience, however, has 35 not borne out such an assumption. The differ-

ences between magnesium base and aluminum base—magnesium alloys are well defined. For example, magnesium base alloys are only attacked on the surface when cast in green sand molds whereas aluminum base-magnesium alloys develop a sub-surface oxidized zone which cannot be seen by ordinary visual inspection. In commercial practice different types of sand are used in making sand molds for the casting of magnesium and aluminum base alloys, a coarse porous sand being employed for the former kind of alloys and a fine grained sand for the latter variety of alloy. This difference in the sand used necessitates different molding practices, and what might be effective in treating one type of sand would not be adapted to use in the other type. A further distinction between the two kinds of base alloys lies in the difference in response to substances intended to inhibit oxidation. Sulphur, for example, which has been commonly used in sand molds for the production of magnesium base 40 alloy castings is entirely ineffective in preventing the formation of frame in an aluminum base—magnesium alloy casting. Other substances also, such as urea, which are satisfactory for protecting magnesium base alloys afford little or no protection against the occurrence of frame in aluminum base—magnesium alloys. As a result of my investigation it may be safely said that no prediction can be made as to the behavior of one type of alloy in the presence of a protective substance, from the action of the same substance upon the other type of base alloy.

One of the objects of my invention is to inhibit the formation of frame in aluminum base—magnesium alloys that are cast in green sand molds. Another object is to incorporate a substance in the molding sand which will not only inhibit the formation of frame but will not destroy the molding quality of the sand. Still another object is 45 to employ a substance in the manufacture of sand molds which is not volatile at ordinary temperatures and does not react with the water used to temper the sand. A further object is to use a substance that does not yield noxious fumes in contact with the molten metal in the mold.

I have found after an extended investigation that the incorporation of from about 1 to 10 per cent of ammonium fluoride in molding sand tempered with water effectively inhibits the formation of frame in aluminum-magnesium alloys cast in molds made from such a mixture. If desired, the mold may be first made in the usual manner without mixing any ammonium fluoride with the sand, and then the surface of the mold 50

cavity may be treated by spraying with a solution of the salt or simply dusting the walls with the powdered salt prior to pouring metal therein. I have found it advantageous to employ an alcoholic solution of ammonium fluoride for spraying purposes and allow the solvent to evaporate before introducing the metal into the mold. Such easily vaporizable alcohols as methyl alcohol and ethyl alcohol are satisfactory solvents of ammonium fluoride. The inhibitive effect of the ammonium fluoride is the same whether it is mixed with the sand or merely sprayed on the surface of the mold. The manner of using the protective agent will in any case depend upon the nature and number of castings to be made. Where only a few castings are desired, it is obvious that it would be more economical to coat the mold cavity than to incorporate the salt with the sand mixture.

20 The sands used in making green sand molds, where my invention is practiced, are tempered with about 4 to 9 per cent of water; that is, just enough water is added to the molding sand mixture to make it cohesive when molded. The other components of the mixture need not be varied on account of the use of ammonium fluoride, since the salt does not destroy the cohesion of the molding mixture.

30 The merits of my invention may be illustrated through reference to some comparative tests which have been made. An aluminum-magnesium alloy containing about 6 per cent magnesium, balance aluminum, was cast in the usual 35 type of green sand mold made from a molding mixture of silica grain sand and clay tempered with about 6 per cent water. A fracture of the casting showed that a black ring or reaction zone had been produced immediately below the surface, which was not visible from the surface by ordinary inspection. Another portion of the same alloy was cast in the same kind of mold which had been sprayed with a 4.2 per cent methyl alcohol solution of ammonium fluoride and the alcohol

40 allowed to evaporate before the metal was introduced. No black ring appeared on the latter casting except in a portion of the gate. The useful part of the casting, however, was clean and bright. The deleterious effect of such a ring upon the 45 physical properties of a cast article is shown by a comparison of the properties of the aforementioned castings. The castings made in the untreated mold had an average tensile strength of 23,400 pounds per square inch, a yield strength of 50 14,000 pounds per square inch, and an elongation of 6.3 per cent in two inches. Castings made in the second, or treated mold, in marked contrast, had an average tensile strength of 27,800 pounds per square inch, a yield strength of 55 15,400 pounds per square inch, and an elongation of 8.4 per cent in two inches.

60 In preparing a mixture of molding sand and ammonium fluoride, I prefer to use from about 2 to 6 per cent of the salt and temper the mass 65 with 5 to 7 per cent of water. In general, when the water content of the sand is near the maximum allowable amount, a greater quantity of ammonium fluoride should be used as a precaution against the reaction with the water. If the 70 salt is sprayed on the surface of the mold cavity either an aqueous or an alcoholic solution may be employed, but in practice I prefer the alcoholic solvent because of its greater volatility. The use

of such a solvent avoids the introduction of more water into the mold, and upon evaporation it leaves a layer of ammonium fluoride on the walls of the mold cavity. Under some conditions a simple dusting of the mold walls with the powdered salt may provide sufficient protection against formation of the black ring. The essential feature of my invention, in any case, is that ammonium fluoride shall be brought into contact with the molten aluminum-magnesium alloy, 5

10 While my invention is applicable to aluminum base alloys containing more than 50 per cent aluminum, it is especially effective in alloys containing between about 4 and 15 per cent magnesium, the range usually employed in the manufacture of aluminum-magnesium alloy castings. Alloys containing this amount of magnesium reveal the black sub-surface ring described hereinabove when said alloys are cast in the usual green 15 sand mold.

20 I claim:

1. A method of making castings of aluminum base alloys containing from about 4 to 15 per cent magnesium in green sand molds, comprising 25 bringing ammonium fluoride in contact with the surface of the molten metal next to the mold walls.

2. A method of making castings of aluminum base alloys containing from about 4 to 15 per cent magnesium in green sand molds, comprising 30 tempering the molding mixture with from about 5 to 7 per cent water, forming the mold, treating the walls of the mold cavity with ammonium fluoride, and casting the metal in said 35 mold.

3. A method of making castings of aluminum base alloys containing from about 4 to 15 per cent magnesium in green sand molds, comprising 40 adding from about 1 to 10 per cent of ammonium fluoride to the molding mixture, tempering the mixture with from about 5 to 7 per cent water, forming the mold, and casting the metal therein.

4. A green sand mold for casting aluminum base alloys containing from about 4 to 15 per cent magnesium, said mold being made from a molding mixture tempered with about 5 to 7 per cent water, and the walls of said mold being 45 treated with ammonium fluoride prior to the introduction of the metal.

5. A green sand mold for casting aluminum base alloys containing from about 4 to 15 per cent magnesium, said mold being made from a molding mixture containing from about 1 to 10 50 per cent ammonium fluoride, and tempered with 5 to 7 per cent water.

6. A method of making castings of aluminum base alloys containing from about 4 to 15 per cent magnesium in green sand molds, comprising 60 adding from about 1 to 10 per cent of ammonium fluoride to the molding mixture, tempering said mixture with from about 4 to 9 per cent of water, forming the mold, and casting the metal in said mold.

7. A green sand mold for casting aluminum base alloys containing from about 4 to 15 per cent magnesium, said mold being made from a molding mixture containing from about 1 to 10 70 per cent ammonium fluoride, and tempered with 4 to 9 per cent water.

ROY E. PAINE.